

June 7, 1932.

S. BOYER

1,862,366

MARKING QUARTZ

Filed March 2, 1926



Inventor:  
Sylvester Boyer,  
by *Alfred S. Lunt*.  
His Attorney.

## UNITED STATES PATENT OFFICE

SYLVESTER BOYER, OF LYNN, MASSACHUSETTS, ASSIGNOR TO GENERAL ELECTRIC COMPANY, A CORPORATION OF NEW YORK

## MARKING QUARTZ

Application filed March 2, 1926. Serial No. 31,843.

My present invention relates to means for marking quartz and more particularly to means for marking quartz which may be subjected to relatively high temperatures, such 5 as quartz thermometers of the type disclosed in my copending application, Serial No. 70,191, filed November 19, 1925.

The marking of a thermometer or glass vessel of any type usually comprises two steps, 10 first the etching of a mark on the glass, and second the placing of a contrasting material on the etched mark whereby the position or character of the mark may be made clearly visible. The marking of quartz, however, 15 involves certain difficulties. For example, it has hitherto been impossible to etch fused quartz so as to produce a clearly defined line or design thereon. Attempts to etch quartz by well known methods, as by coating the 20 quartz with paraffin and producing a mark through the paraffin on the quartz and then placing the coated quartz in cold or unheated hydrofluoric acid, have resulted uniformly in failure due to the fact that the etching produced in such cases extends, as a rule, over 25 the entire surface of the quartz, and is not confined to the marked places. Further difficulty is encountered in marking quartz which is subjected to relatively high temperatures, 30 as in the case of quartz thermometers, since it is necessary that such marks should be colored in order to be clearly visible, and should furthermore be capable of withstand- 35 ing the high temperatures encountered in the use of such thermometers without causing discoloration of the quartz body.

It is one of the objects of my invention to provide a marking on quartz which shall be sharply defined, clearly visible, stable, and 40 permanent in character even when exposed to temperatures in the neighborhood of 1000° C.

The accompanying drawing shows in elevation a quartz thermometer embodying the features of my invention.

45 The quartz thermometer 1 may be provided with a central bore 2 having a bulb 3 adapted to contain a quantity of gallium or other suitable material. I preferably employ in connection with the thermometer an expansion chamber as indicated at 4, for pur-

poses clearly set forth in my above cited co-pending application. At different points on the stem of the thermometer, indicating marks are placed, as clearly shown on the drawing. These marks may be placed at 55 suitable distances apart to suit convenience and may be placed on the stem following the filling of the thermometer with the expandible material.

To produce a sharply defined etched mark 60 on the quartz, hydrofluoric acid, preferably dilute, and heated to a temperature of approximately 80° C., may be conveniently employed. Since the paraffin coating usually employed in etching glass would melt far 65 below such a temperature, it is necessary to employ a protective coating for the quartz which will remain on the quartz body at least for the duration of the etching period.

In the process employed, the quartz is first 70 cleaned in any suitable manner and then heated either in a free flame or oven to a dull redness. The quartz is then immersed in a polymerizable or oxidizable material, such as chinawood or linseed oil, or, if de- 75 sired, a japan varnish, and allowed to remain therein for a relatively short period of time, for example, one or two minutes, or until any possible film of air on the quartz surface has been completely replaced by the oil. The 80 quartz is now removed from the oil and held above a free flame or heated in an oven until a distinct coloration occurs indicating that polymerization has taken place. The degree of polymerization will vary with the type 85 of marking desired on the quartz. If a very fine mark is desired, the oil is polymerized to the extent of becoming quite hard, while if a rather wide mark is desired the polymerization should not be carried so far. Marks 90 are now made through the oil coating and on to the quartz surface, the marks penetrat- 95 ing the quartz surface only to a very slight extent, since etching will take place more quickly and satisfactorily if the surface of the quartz is only slightly scratched, than where a relatively deep mark is made. The quartz is now placed in dilute hydrofluoric acid, which is heated to 80 or 90° C. for a period of time which may vary from 5 to 20 100

minutes, depending on the nature of the mark desired. If a mark having sharp edges is desired, a period of from 8 to 10 minutes will prove satisfactory, while if a mark having a rounded edge is desired, the quartz should be exposed to the acid for a longer period of time. After the quartz has been acted upon by the acid for a suitable time, it is taken out of the acid and the oil coating removed. This may be easily accomplished as the oil coating usually tends to become loosened from the quartz surface during the latter portion of the etching operation.

In order to make the etched mark on the quartz clearly visible, it is necessary to place on the etching some colored material. If the quartz is to be employed in the measurement of high temperatures, it is also essential that the coloring matter be stable under high temperature conditions. I have found that a very desirable grayish black mark may be produced by a quantity of copper oxide and fine sand or silica suspended in glycerine. About six parts of the oxide and one part silica when added to sufficient glycerine to produce a material which may be used as an ink, gives a very satisfactory mixture. The liquid may be placed on the etched portion of the quartz with an ordinary pen or in any other suitable manner, although it will be found that a specially prepared pen which will more or less confine the liquid to the etched portions will give the best results. The marked portion of the quartz is now held above a free flame and heated slightly to evaporate the glycerine. Evaporation should be carried out slowly in order to confine the colored material within the etched mark. After the glycerine is driven off the quartz is heated in the oxidizing portion of a free flame to redness, or until fusion of the oxide, silica, and quartz is complete.

Quartz marked in the manner described above has been subjected to temperatures as high as 1100° C. for relatively long periods of time without causing deterioration of the markings or any discoloration of the quartz body. I have, furthermore, found such a marking to be insoluble in the ordinary laboratory reagents, such as hot and cold sodium hydroxide, hot and cold nitric acid, hydrochloric acid and aqua regia.

If desired another colored mark may be obtained by the use of a mixture comprising five parts lead oxide (litharge), one part silica, and about 35 parts cobalt oxide, suspended in glycerine and placed on the etched portion of the quartz and heated as above described. The proportions of the oxides given may vary considerably without showing marked changes in the final result. If desired, a green marking may be obtained by taking a mixture comprising three parts lead oxide, one part silica and about 28 parts barium chromate, suspended in glycerine,

placing the liquid mixture on the etched mark and heating in the manner previously set forth.

What I claim as new and desire to secure by Letters Patent of the United States is:

1. A thermometer formed from fused quartz and having vitreous contrasting markings fused thereon, said markings being composed of material which is stable at a temperature up to and in excess of 500° C.

2. A thermometer formed from fused quartz and provided with markings on the surface thereof, said markings being composed of colored vitreous silica fused on said surface and being stable up to and at a temperature of approximately 1,000° C.

3. An article of manufacture formed from fused quartz and provided with markings on the surface thereof, said markings being composed of colored vitreous silica fused on said surface and being stable up to and at a temperature of approximately 1,000° C.

In witness whereof, I have hereunto set my hand this 26th day of February, 1926.

SYLVESTER BOYER.

95

100

105

110

115

120

125

130